

## UNITED STATES PATENT OFFICE.

GEORGE J. NIKOLAS, OF CHICAGO, ILLINOIS.

## METHOD OF FINISHING SICCATIVE COATINGS.

No Drawing.

Application filed May 3, 1923. Serial No. 636,498.

*To all whom it may concern:*

Be it known that I, GEORGE J. NIKOLAS, a citizen of the United States of America, and a resident of Chicago, county of Cook, and

5 State of Illinois, have invented a new and useful Improvement in Methods of Finishing Siccative Coatings, of which the following is a specification.

This invention relates to methods of finishing siccative coatings, as lacquer enamels and the like, for instance, on metal, wood or other structural material, especially where the spray-brush or air-brush method is used for applying the coatings. Incident to methods 10 now extensively used, the application of coatings by a spray-brush results in a minutely rough or undulatory surface commonly known as an "orange-peel" effect. In order to remove this defect it is customary to rub down not only the filler coat but also the intermediate coat or coats, as well as the finish coat of lacquer. This leaves a dull finish requiring another coat to give the desired gloss. This last coat also has the defect, i. e., "orange-peel" appearance.

The main object of this invention is to bring up a high finish gloss such as usually is obtained with varnish, and to accomplish this without leaving a surface having 25 the "orange-peel" effect.

My method of accomplishing the above result, where the coatings have been applied by an air-brush, or where for any other reason they have an "orange-peel" surface, is to 30 rub down the finish with some abrasive to remove the "orange-peel" effect; then I apply a thinner to the coated object, which is otherwise finished, and I let this drain off. The thinner, commonly known as a lacquer thinner, may be either poured on the object to 35 be treated, or it may be sprayed on, or if pre-

ferred the object may be immersed or dipped briefly in a bath of thinner material. For this purpose I use a nitro-cellulose solvent, or such a solvent mixed with a diluent.

The effect of the thinner is to soften the surface of the coating which probably due to surface tension, then assumes a perfectly smooth exterior, and upon drying and setting, requiring but a brief interval, presents the smooth high gloss finish which is considered essential for most finishes of the character referred to, as for instance, on automobile bodies, and other objects requiring a high grade coating finish.

Although but one specific embodiment of the process of this invention is herein described, it is to be understood that some of the specific steps may be modified or omitted without departing from the spirit of this invention as defined by the following claims.

I claim:

1. The method of finishing a siccative coating which includes applying a thinner thereto after the coating has dried.

2. The method of removing orange-peel effects from coatings which includes the application and draining off of a thinner.

3. The method of bringing up a gloss finish on a coating after it has been rubbed down, which consists in applying briefly thereto a nitro-cellulose solvent.

4. The method of coating and finishing an object which consists in applying a siccative coating thereto, then after the coating has dried, rubbing it down to remove the orange-peel effect, and then applying briefly thereto a thinner to bring up a gloss finish.

Signed at Chicago this 5th day of February, 1923.

GEORGE J. NIKOLAS.